

## UNITED STATES PATENT OFFICE.

WILLOUGHBY STATHAM SMITH, OF NEWTON POPPLEFORD, HENRY JOSEPH GARNETT, OF SEVENOAKS, AND JOHN ANCEL HOLDEN, OF GIDEA PARK, ENGLAND.

## ALLOY AND ITS APPLICATION TO THE MANUFACTURE OF ELECTRICAL CONDUCTORS.

No Drawing. Application filed January 6, 1927, Serial No. 159,497, and in Great Britain July 10, 1926.

The subjects of this invention are quaternary alloys of iron, nickel, aluminium and a variable fourth element. As a fourth element, chromium has been found to be particularly advantageous, as suitable alloys of these four metals are characterized by their high electrical resistances and their very high permeabilities with very weak magnetizing forces. Other metals desirable as a fourth element are molybdenum, vanadium, tungsten and silicon.

A feature of this invention is that whereas in nickel-iron-aluminium alloys (in which nickel predominates and where the aluminium exceeds 3%) forgeability is difficult, in the quaternary alloys herein described this difficulty does not exist.

According to this invention a quaternary alloy free from carbon comprises:

|                    | Per cent. |
|--------------------|-----------|
| Iron               | 6-17      |
| Aluminium          | 1-5       |
| A fourth element   | 1-5       |
| Nickel the balance |           |

Although these alloys are termed quaternary alloys, yet they may contain a small percentage of a deoxidizing metal, such as manganese, cadmium or magnesium.

To obtain the highest resistance and the highest initial permeability the percentages can be still more narrowly defined as

|                                           | Per cent. |
|-------------------------------------------|-----------|
| Iron                                      | 8-11      |
| Aluminium                                 | 2-3       |
| A fourth element                          | 2-3       |
| Nickel the balance, but not less than 84% |           |

Thus an alloy containing:

|                    | Per cent. |
|--------------------|-----------|
| Iron               | 9.5       |
| Aluminium          | 2.8       |
| Chromium           | 2.8       |
| Manganese          | .1        |
| Nickel the balance |           |

when forged, drawn to wire and annealed at 900° C. had the following properties:

Electrical resistance 67.5 microhms per cm<sup>3</sup>. Initial permeability 8000.

An alloy free from carbon containing:

|           | Per cent. |
|-----------|-----------|
| Iron      | 17.0      |
| Aluminium | 2.0       |
| Chromium  | 1.5       |

and the balance nickel, when forged, drawn to fine wire and annealed at 900° C. gave a permeability of 8000 in a field of .001 gauss and 11,500 in a field of .1 gauss together with an electrical resistance of 44.4 microhms per cm<sup>3</sup>.

When either the aluminium or the fourth element is given a content approaching its maximum content, the magnetic permeability of the alloy in weak fields will be very considerably reduced, but the fall will not be so great if the iron content approaches the minimum iron content i. e. 6%. Thus an alloy containing:

|                    | Per cent. |
|--------------------|-----------|
| Iron               | 6         |
| Aluminium          | 2.8       |
| Chromium           | 5         |
| Nickel the balance |           |

forged, drawn to wire and heat treated had an initial permeability of 3000 and an electrical resistance of 80 microhms per cm<sup>3</sup>.

These alloys are very sensitive to heat treatment and in those applications where minimum hysteresis is a very important factor, such as for the wires and tapes used in submarine telegraph cable systems, great care is necessary not to over anneal the alloys. For fine wire (from 30 to 40 standard wire gauge) thin stampings (.006 inches to .020 inches thick) two minutes annealing at 880° C. in an inert atmosphere, such as nitrogen, followed by rapid cooling, will develop the magnetic permeability and the hysteresis will be almost negligible.

What we claim is:

- An alloy free from carbon composed of 6 to 17% iron, 1 to 5% aluminium, 1 to 5% of a fourth metal for increasing the electrical resistance and selected from a group comprising chromium, molybdenum, tungsten, vanadium, or silicon and the balance nickel.
- An alloy free from carbon composed of 6 to 17% iron, 1 to 5% aluminium, 1 to 5% chromium, and the balance nickel.
- An alloy free from carbon composed of 6 to 17% iron, 1 to 5% aluminium, 1 to 5% of a fourth metal for increasing the electrical resistance and selected from a group comprising chromium, molybdenum, tungsten, vanadium, or silicon, a small percentage of a deoxidizing metal, and the balance nickel.
- An alloy free from carbon composed of

6 to 17% iron, 1 to 5% aluminium, 1 to 5% chromium, a small percentage of a deoxidizing metal, and the balance nickel.

5. An alloy free from carbon composed of

6 to 17% iron, 1 to 5% aluminium, 1 to 5% of a fourth element for increasing the electrical resistance and selected from a group comprising chromium, molybdenum, tungsten, vanadium, or silicon, a small percentage of manganese, and the balance nickel.

6. An alloy free from carbon, composed of 6 to 17% iron, 1 to 5% aluminium, 1 to 5% chromium, a small percentage of manganese, and the balance nickel.

15 7. An alloy free from carbon composed of 6 to 17% iron, 1 to 5% aluminium, 1 to 5% of a metal in Class VI of the periodic system, and the balance nickel.

8. An alloy free from carbon composed of 20 6 to 17% iron, 1 to 5% aluminium and 1 to 5% of a metal in Class VI of the periodic system, a small percentage of a deoxidizing metal, and the balance nickel.

9. An alloy free from carbon composed 25 of iron 8 to 11%, aluminium 2 to 3% and a fourth metal 2 to 3%, said metal increasing the electrical resistance and being selected from a group comprising chromium, molyb-

denum, tungsten, vanadium, or silicon, and the balance nickel, but, however, not less than 84%.

10. An alloy free from carbon composed of iron 8 to 11%, aluminium 2 to 3% and a fourth metal 2 to 3%, said metal increasing the electrical resistance and being selected from a group comprising chromium, molybdenum, tungsten, vanadium, or silicon, a small percentage of a deoxidizing metal, and the balance nickel, not, however, less than 84%.

11. An alloy free from carbon composed of iron 8 to 11%, aluminium 2 to 3% and chromium 2 to 3%, and the balance nickel, not, however, less than 84%.

12. An alloy free from carbon composed of iron 8 to 11%, aluminium 2 to 3%, and a metal in Class VI of the periodic system 2 to 3%, and the balance nickel, not, however, less than 84%.

In testimony that we claim the foregoing 50 as our invention, we have signed our names this 21st day of December, 1926.

WILLOUGHBY STATHAM SMITH.  
HENRY JOSEPH GARNETT.  
JOHN ANCEL HOLDEN.